

Oct. 29, 1935.

S. D. WELLS

2,018,938

APPARATUS FOR AND METHOD OF TREATING AND HANDLING  
PAPER PULP AND SIMILAR FIBROUS MATERIALS

Filed Jan. 9, 1933

3 Sheets-Sheet 1



Oct. 29, 1935.

S. D. WELLS

2,018,938

APPARATUS FOR AND METHOD OF TREATING AND HANDLING  
PAPER PULP AND SIMILAR FIBROUS MATERIALS

Filed Jan. 9, 1933

3 Sheets-Sheet 2



INVENTOR.

*Sidney D. Wells*

BY  
*Batten, Thedwell, Lester,  
McNamee & Milne*

ATTORNEYS

Oct. 29, 1935.

S. D. WELLS

2,018,938

**5. S. D. WELLS**  
APPARATUS FOR AND METHOD OF TREATING AND HANDLING  
PAPER PULP AND SIMILAR FIBROUS MATERIALS  
Filed Jan. 9, 1933 3 Sheet

AND SIMILAR PLATES  
Filed Jan. 9, 1933

3 Sheets-Sheet 3



INVENTOR.

Sidney D. Wells

BY *Bettine, Hudacek, Lecker,  
McNamara & Michael*  
ATTORNEYS

## UNITED STATES PATENT OFFICE

2,018,938

APPARATUS FOR AND METHOD OF TREAT-  
ING AND HANDLING PAPER, PULP AND  
SIMILAR FIBROUS MATERIALSSidney D. Wells, Appleton, Wis., assignor to  
Lewis L. Alsted, Appleton, Wis.Continuation of application Serial No. 619,863,  
June 29, 1932. This application January 9, 1933,  
Serial No. 650,935

19 Claims. (Cl. 92—9)

This invention relates generally to an apparatus for and a method of treating or handling paper pulp or similar fibrous materials and is particularly designed and adapted for de-inking paper that has been printed upon. For example, it may be used with special advantage for the purpose of removing from paper, containing ground wood pulp, ink in which carbon black has been used as the pigment. In this connection it has been proposed to remove printing ink from paper by subjecting such paper to the action of naphtha soap and soft water and then resorting to simple filtration to separate the loosened carbon particles from the fiber, the carbon particles passing off with the filtrate. Such a method forms the subject matter of Patent 1,826,179, granted October 6, 1931, to Minnie E. and Bruce W. Kinyon.

This application is a continuation of and a substitute for my pending application for apparatus for and method of removing printing ink from paper, filed June 29, 1932, Serial No. 619,863.

The method of the present invention differs from the Kinyon process and other prior processes and practices in that it does not depend for its efficacy upon the use of any specific solvent or detergent but relies rather upon a novel physical-chemical action and is advantageous over such prior practices in that a more complete removal of the ink is effected and this with substantial economies in the use of the soap or solvent. In general, the present method is more efficient and better lends itself to commercial operations on a large scale.

Broadly, the present method of removing printing ink from paper comprises disintegrating the paper and agitating it in a soapy solution until the ink is loosened from the paper and a foamy mass, containing substantially no free liquid, is produced. Such a mass is constituted of the paper fibers and innumerable soap bubbles interspersed therebetween. During the production of the mass the soapy solution emulsifies or dissolves the binder or vehicle used in the ink and the pigment of the ink is reduced to a powder or multiplicity of carbon particles. These carbon particles are taken up by the films of the soap bubbles. The carbon black used as a pigment in printer's ink is readily wet by the soap solution and has a greater affinity for the soap films of the foamy mass than it has for the pulp fibers. After once being removed in this manner from the pulp fibers there is no longer any tendency for the carbon to attach itself to them again.

The next essential step in the process is the separation of the bubbles with the pigment particles thereon from the fibers and this is accomplished by subjecting the mass to the action of a de-watering or de-liquoring device of the type known in the art as a screw press. In the screw press the mass is squeezed or pressed and the soap bubbles with the carbon particles thereon are expressed or extruded through the screen of the press leaving clean white fibers behind. The presence of the soap bubbles precludes the fibers from felting or matting together and thus forming a filtering medium, and the bubbles, on account of their elasticity, are capable of changing their shapes and following the irregular passages through the mass. The use of a screw press is especially advantageous in that it applies the positive force in just the manner required to effect separation of the foam or bubbles from the fiber. Any attempt to effect this separation by rinsing or washing will break the films and allow the carbon particles to redeposit on the fibers. Furthermore, the advantage of reducing the power requirements is had. When a good foam condition exists the power requirements of the screw press are reduced from 50% to 70% on account of the lubricating effect of the soap films and air bubbles. This feature possesses utility apart from the method herein disclosed and in its broader aspects consists in the employment of foam or soap bubbles to aid in the handling of pulp. For this general purpose the feature has the same advantage of reducing the power requirements.

Commercially, it is usually desirable to repeat the steps of the process several times at least. Preferably, a rod mill is used to disintegrate and agitate the paper in its soapy solution in the first instance. The employment of a rod mill for this purpose is especially advantageous in that it makes possible to use only four parts of water to one part of fiber, whereas with types of apparatus heretofore proposed for similar purposes it was necessary to use at least sixteen parts of water to one part of fiber. The use of one quarter of the water means that only one quarter of the chemicals required to produce a given concentration need be used, and similarly only one quarter of the steam ordinarily required is here essential to produce a given temperature. Finally, only one quarter of the power ordinarily needed to produce a given amount of maceration or working is necessary with the rod mill. Where the steps of the process are repeated then the subsequent

acts of producing the foamy mass may usually be more conveniently carried out in simpler and less expensive types of devices, as, for example, what are known as mixing conveyors. Mixing conveyors consist simply of a tank or some sort of a receptacle in which twin screws, revolving flights or similar devices operate to intimately mix the solution or effluent with the pulp cake delivered thereto from the first screw press and thereby 10 produce a foamy mass similar to that which entered the first screw press but which, of course, contains less carbon particles.

One way of advantageously carrying out the method on a commercial scale consists in utilizing 15 a rod mill to effect the disintegration and the initial production of the foamy mass, then expressing approximately 75% of the foamy mass from the fibers by passing the mass through a screw press, then again beating and agitating the 20 resultant cake from the screw press in a mixing conveyor and in the environment of more soapy solution, again expressing a portion of the soap bubbles from the resultant foamy mass in a screw press and repeating this remixing and separation 25 until the fibers are practically free of the pigment. The final step in the process consists in washing the cake of fibers and soap bubbles with water. This may be done in a mixing conveyor and this final step is completed by expressing a 30 substantial portion of the water from the fibers in a screw press. During the cycle of operations, the rod mill, screw presses and mixing conveyors are so connected up in the system that the soapy solution is gaining the ink pigment as it travels 35 back to the first stage of the process and the fiber is losing ink pigment as it approaches the final stage of the process. This is effected by introducing clear water into the system at the final stage or washing stage, then carrying the water 40 which is expressed from the fibers back to the next to the last stage. The water so carried back contains, of course, some proportion of soap in solution. The effluent from the next to the last stage is then carried back to the second stage of 45 the process and during its travel back is supplied with soap in sufficient quantity to incorporate in the solution the desired percentage of soap. From the second stage the effluent is carried back to the rod mill or the first stage. The solution or 50 effluent which is expressed from the foamy mass in the first stage is carried off to any suitable point of discharge.

Soap stocks are selected which foam readily and which contain relatively high amounts of 55 oleic acids. Saponin may also be employed. As will be understood, saponin is a glucoside derived from vegetable fibrous material and has an ability to produce foam many times as great as that of the most efficient soaps. However, the utmost 60 economy in practicing the method may be realized by using spent cooking liquors recovered from the digestion of fibrous material as the foam producing material. In this connection, it should be understood that in the treatment of 65 fibrous vegetable materials for the liberation of the fiber the incrusting matter consisting of albumenoids, pentosans, glucosides, resin, lignins and similar substances are more or less dissolved and are removed in the washing. Many of the 70 substances are copious foam producers, especially in the combination in which they exist in the spent cooking liquors and these liquors in the condition in which they exist after the fiber washing 75 operation or after proper modification can be

used for purposes where foam producers are needed.

For instance, the liquors obtained from the cooking of extracted licorice root are copious foam producers without further modification. Liquors 5 from the mild digestion of corn stalks with caustic soda are also copious foam producers.

In the digestion of resinous woods by the sulphate process considerable quantities of resin soaps occur in the spent liquors. These soaps are 10 largely emulsified so that by the concentration of the liquors so that their specific gravity differs substantially from the gravity of the soaps the latter may be separated by the application of centrifugal force by means of centrifuges as, for instance, the well known cream separators.

Products from the bleaching of kraft pulps which are washed out are copious foam producers. The spent liquors from sulphite cooking have also this characteristic. By the substitution of sodium for the calcium radical the foam producing properties may be enhanced and particularly where the subsequent reaction must take place in the neutral or slightly alkaline state. Each substance has an optimum pH which can be found by 20 trial. The materials or soaps used must have detergent properties as well as foam producing properties. Naphtha soap might be used but care must be taken that naphtha not be used in excess as when so used it tends to retard the foam- 25 ing properties of the soap. The use of naphtha soap is especially desirable in hard water as with hard water calcium and magnesium soaps are formed and they tend to impair the capacity of the solution to wet the carbon particles and set up 30 a condition where the carbon particles tend to redeposit on the fibers. This adverse tendency may, however, be overcome by using an excess of soap and especially so by using soft water.

As to the amount of soap, from 7% to 10% of 40 the weight of the paper stock added to the effluent from the third press will give good results. About 5% of the weight of the paper stock of bentonite added to the water supplied to the fourth press will further improve results and 45 prevent coagulation of the soap that remains in the pulp when it is necessary to use hard water in the paper making operation that follows. Room temperature or approximately 65° F. is satisfactory for carrying on the reaction although 50 heating to 130° F. may slightly improve the results. The invention also contemplates the use of alkalis such as caustic soda in dilute solution to loosen the ink from the paper and in combination therewith a foam producing substance such as 55 some synthetic soaps commercially available which are capable of exerting foam producing properties throughout a wide range of acidity or alkalinity.

The accompanying drawings illustrate one type 60 of apparatus which may be used to carry out the process and in the drawings:

Figure 1 is a diagrammatic view illustrating one way of connecting up the instrumentalities utilized to carry out the method;

Figure 2 is a perspective view showing one type 65 of rod mill which may be used to carry out the present method;

Figure 3 is a view in perspective with parts 70 broken away and shown in section to further illustrate the rod mill;

Figure 4 is a view in longitudinal vertical section showing a screw press utilized in carrying 75 out the method; and

Figure 5 is a sectional view illustrating diagrammatically one type of mixing conveyor which may be employed.

Referring to the drawings, it will be seen that the apparatus utilized for carrying out the method includes a rod mill designated generally at 1. The rod mill is of conventional construction and has the usual rotating cylinder 2 containing the rods 3. The paper is fed in through the inlet 4 of the cylinder and discharged from the outlet 5.

The rod mill is supplied with a soapy solution by means of a pipe 20 which connects with the screw press 19 used in the second stage of the process and carries the effluent from this screw press 19 into the rod mill. The action of the falling rods in the rod mill upon the old newspaper or other paper stock and the soap solution results in the formation of a foamy mass so that the comminuted or fibrous material which emerges from the discharge end of the mill contains innumerable minute bubbles. During the treatment in the rod mill, the soapy solution emulsifies or dissolves the binder or vehicle used in the ink and the pigment is reduced to a powder or a multiplicity of particles which is taken up by the films of bubbles as above described.

The discharge from the rod mill is carried by conveyors or by any suitable means to a screw press designated generally at 7. In the diagram for the purpose of simplicity in illustration the means for carrying the discharge from the rod mill to the screw press is shown diagrammatically as a pipe 6.

The screw press 7 is also of conventional construction and comprises an outer casing 8, a cylindrical screen 9 in spaced relation to the inner wall of the outer cylinder, and a screw 10. The depth and pitch of the thread of a screw varies from the inlet to the outlet and so that as the foamy mass from the rod mill is fed through the screw press a certain percentage of bubbles will be forced out through the screen 9 and pass on to the point of discharge through the pipe 11. The rod mill and screw press constitute the first stage of the particular process being exemplified and in these two instrumentalities the essentials of the fundamental process are carried out, that is to say, the paper is disintegrated and agitated in a soapy solution to produce a foamy mass containing substantially no free liquid in which there are innumerable bubbles carrying the ink pigment and thereafter the bubbles with the pigment are expressed from the fibers.

As pointed out, however, it is usually desirable in actual practice to repeat this fundamental process, that is, to refoam the cake which is extruded from the screw press of the first stage and again express soap bubbles containing pigment particles from the fibers.

In carrying out this repetition, the cake from the first screw press 7 which consists of fibers with a certain amount of soap bubbles are carried through a pipe 12 or by any other suitable conveying means into a mixing conveyor 13. The mixing conveyor may consist of a suitable tank in which twin screws, revolving flights or similar devices, illustrated diagrammatically at 14, operate and function to intimately mix the cake delivered thereto with the soapy solution or effluent delivered thereto. Because the cake is wet the action does not have to be as vigorous as that given by the rod mill where the waste paper first enters the system. It will be noted as the description proceeds that a counter-flow principle of circulating the solution through the system is

resorted to in order that the solution or effluent may gain ink as it travels back through the first stage of the treatment and that the pulp or fibers may lose ink as they approach the final stage of the process. In other words, the dirtiest solution is working on the dirtiest paper and the cleanest solution on the cleanest paper. In fact, this is carried out to such extent that clear water washes the fibers in the final stage. In carrying out this purpose, the solution supplied to the mixing conveyor 13 of the second stage is the effluent from the screw press 15 of the third stage reinforced with a proper amount of fresh soap stock or soap solution. As shown in Figure 1, a pipe 16 leads from the discharge of the screw press 15 of the third stage and discharges into a soap supply means 16'. After picking up the proper amount of fresh soap stock the effluent passes on through a pipe 17 to the mixing conveyor 13 of the second stage.

After the process has been carried to such an extent as to produce in the mixing conveyor 13 a foamy mass devoid of free liquid it is carried by any suitable means, as by pipe 13', to a second screw press designated at 19 in which it is pressed and further relieved of the solution and impurities. Leaving the screw press 19, the cake of fibers with some soap bubbles therein is carried into a mixing conveyor 21 where it is again beaten into a foamy mass. The soapy solution 30 is supplied to the mixing conveyor 21 through a pipe 22 which leads from the screw press 23 of the final or washing stage. Leaving the mixing conveyor 21 the foamy mass is carried through the screw press 15 wherein it is again subjected to pressure to cause the soap bubbles to pass through the meshes of its screen leaving substantially clear white fibers and some soap bubbles behind.

In the final stage which includes the mixing conveyor 25 and the screw press 23, the cake is agitated in and is washed by clear water which is supplied to the mixing conveyor 25 from a pipe 26. After the washing has been carried out to a point sufficient to dissolve out the soapy bubbles the resulting mass is transferred to the screw press 23 and in the screw press the soap solution is separated from the fibers and is carried back to the mixing conveyor 21 of the third stage as just described.

The soap bubbles in the cake delivered from the screw press 23 are devoid or practically devoid of any carbon particles. In fact, it is estimated that there is not more than

50

55

12  
12463

parts of the ink originally on the paper in the fibers delivered from the apparatus.

This estimate is based on the utilization of four screw presses connected up in the system in accordance with the counterflow principle hereinabove described and on supplying to the rod mill one part of paper to eleven parts of water. Under these conditions, the foamy mass entering each screw press contains, of course, eleven parts of water to one of fibers and leaves the screw press containing two parts of water to one of fiber. Consequently 80% of the impurities carried by the liquor or foam on entering the press are removed by each pressing.

Usually the best results are obtained when there is substantially no free liquid in the foamy mass but the presence of a certain amount of free liquid does not defeat the purposes of the proc-

75

ess. The expression "substantially no free liquid", as used in the specification and claims, is intended to mean that condition in the foamy mass where there is more of the liquid taken up by the fibers and the bubble films than is free and wherein the bubble films are present in sufficient numbers to take up the free particles of the ink pigment. There should not be sufficient free liquid in the mass to break down the bubbles or interfere with their capacity of taking up the particles of the pigment.

It is to be understood that the invention is not limited to the particular number of treatments or stages described. The particular system described has been selected merely for the purpose of illustration. Any desirable number of treatments may be resorted to provided the paper is disintegrated and worked up into a foamy mass in a soap solution so that the particles of pigment are deposited on the surfaces of the bubbles and not on the fibers and may be readily separated from the fibers. In addition to this broad novelty, there are, however, additional advantages in the particular system shown and particularly in the counter-flow principle of circulating the cleansing solution.

Furthermore, while the invention has been described as particularly designed and adapted for use in removing carbon ink pigment from paper stock containing ground wood it is to be understood that the apparatus and method are not restricted to this particular application or use, the present invention being capable of advantageous use for effecting separation from fibrous materials of various other substances or pigments insoluble in water providing that there is a sufficient differential between the degree of attraction of the film surfaces of the bubbles for such substances or pigments and for the fibrous material. The invention has been advantageously employed in recovering clean, fresh pulp of high quality from bleached pulp made from corn stalks but which had been badly damaged by mildew. In such damaged pulp the fruiting bodies, mycelia and spores of the fungi or bacteria had produced black and brown particles of such character and occurrence as to render the pulp unfit for use. By taking such damaged pulp and disintegrating it and agitating it in a solution having detergent and foam producing qualities until a foamy mass containing substantially no free liquid was produced and then by expressing the foam or bubbles from the fibers the objectionable particles were separated from the fibers and a clean, fresh, white pulp of high quality resulted. In this instance just as when the invention was employed to separate the carbon pigment from the pulp containing ground wood, the bubbles or the film surfaces thereof attracted and held the objectionable, non-fibrous particles and when the mass was passed through the screw press the bubbles with the objectionable particles thereon were forced out through the screen leaving the fibers behind. When treating such material the steps of the process are usually repeated and the process is completed by the final washing.

The invention claimed is:

1. The herein-described process of removing printing ink from paper comprising disintegrating the paper and agitating it in a soapy solution until the ink is loosened from the paper and a foamy mass is produced containing substantially no free liquid and having the particles of the ink pigment carried by the films of the bubbles of the

foam and separating the bubbles with the ink pigment thereon from the fibers.

2. The herein-described process of removing printing ink from paper comprising disintegrating the paper in a soapy solution until a foamy mass is produced in which the particles of the ink pigment are carried by the film of the bubbles of the foam and expressing the bubbles with the pigment particles thereon from the fibers.

3. In the art of removing printing ink from paper, the step which consists in disintegrating the paper in a soapy solution until the solution and paper are worked up into a single foamy mass substantially homogeneous throughout and in which the particles of the ink pigment are attracted to and carried by the films of the bubbles of the foam.

4. The herein-described process of removing printing ink from paper comprising disintegrating the paper while subjecting it to treatment with a soapy solution until a foamy mass is produced containing substantially no free liquid and consisting of fibers and innumerable soap bubbles, on the films of which the particles of the ink pigment are held, and expressing the bubbles with the pigment particles thereon from the fibers.

5. The herein-described process of removing printing ink from paper which consists in disintegrating the paper in a soapy solution until a foamy mass is produced in which the particles of the ink are carried by the films of the bubbles of the foam, expressing a portion of the bubbles together with the pigment particles thereon from the mass, and refoaming the mass in a soapy solution and expressing portions of the bubbles together with their pigment particles until the mass is substantially free of ink pigment and finally washing the mass.

6. The herein-described process as set out in claim 5 and further characterized by the utilization of a solution resulting from the washing step for the refoaming step preceding the washing step, and the utilization of the solution which is expressed from the refoamed mass resulting from such refoaming step as the refoaming and foaming solutions for the preceding refoaming and foaming steps.

7. The herein-described process as set out in claim 5 and further characterized by the utilization of a solution resulting from the washing step for the refoaming step preceding the washing step, and the utilization of the solution which is expressed from the refoamed mass resulting from such refoaming step as the refoaming and foaming solutions for the preceding refoaming and foaming steps and in reinforcing one of said refoaming solutions with a fresh supply of soap.

8. In the art of removing printing ink from paper, the step which consists in disintegrating and agitating the paper in a solution having detergent and foam producing qualities until the solution and paper are worked up into a single foamy mass substantially homogeneous throughout and in which the particles of the ink pigment are carried by the films of the bubbles of the foam.

9. The herein-described process of removing printing ink from paper comprising disintegrating the paper in a solution having detergent and foam producing properties until a foamy mass containing substantially no free liquid is produced in which the particles of the ink pigment are carried by the films of the bubbles of the foam and separating the bubbles together with the particles of the ink pigment from the fibers.

10. The herein-described process of removing printing ink from paper comprising disintegrating the paper in a solution having detergent and foam producing properties until a foamy mass is produced in which the particles of the ink pigment are carried by the films of the bubbles of the foam and in expressing from the mass the bubbles together with the pigment particles carried thereby.

11. The herein-described process of removing printing ink from paper which consists in disintegrating the paper in a solution having detergent and foam producing properties until a foamy mass is produced in which the particles of the ink pigment are carried by the films of the bubbles of the foam, expressing a portion of the bubbles together with the pigment particles thereon from the fibers, refoaming the fibers together with the remaining bubbles in a similar solution, again expressing bubbles together with their pigment particles from the refoamed mass, repeating the refoaming and separating steps until the mass is substantially free of ink pigment particles, and finally washing the bubbles from the fibers.

12. An apparatus for removing printing ink from paper comprising means for disintegrating the paper and agitating the same in a soapy solution until a foamy mass is produced consisting of fibers and innumerable soap bubbles on the films of which particles of the ink pigment are carried, means for expressing a portion of said soap bubbles together with the pigment particles thereon from the fibers, means for refoaming the fibers with their remaining soap bubbles, means for separating soap bubbles with pigment particles thereon from the refoamed mass, means for washing the soap bubbles from the fibers following the action of said separating means, and a circulating system for the soapy solution interconnecting said means to cause the soapy solution to travel through the apparatus in a direction counter to that in which the fibers are going whereby to cause the solution to gain and the fibers to lose ink as they pass through the apparatus.

13. An apparatus for removing printing ink from paper comprising a rod mill into which the paper to be treated is fed, means for supplying a solution possessing detergent and foam producing properties into the rod mill whereby the falling rods will disintegrate the paper in the solution and produce a foamy mass containing substantially no free liquid in which the particles of the ink pigment are carried by the films of the bubbles of the foam and means acting on the foamy mass produced by the rod mill to separate the bubbles together with the pigment particles carried thereby from the fibers.

14. An apparatus for removing printing ink from paper comprising a rod mill into which the paper to be treated is fed, means for supplying a solution possessing detergent and foam producing properties into the rod mill whereby the falling rods will disintegrate the paper in the solution and produce a foamy mass in which the particles of the ink pigment are carried by the films

of the bubbles of the foam, and a screw press acting on the foamy mass produced by the rod mill to separate the bubbles together with the pigment particles carried thereby from the fibers.

15. An apparatus for removing printing ink from paper comprising a rod mill into which the paper to be treated is fed, means for supplying a solution possessing detergent and foam producing properties into the rod mill whereby the falling rods will disintegrate the paper in the solution and produce a foamy mass in which the particles of the ink pigment are carried by the films of the bubbles of the foam, a screw press acting on the foamy mass produced by the rod mill to separate the bubbles together with the pigment particles carried thereby from the fibers, means for refoaming the fibers separated from the bubbles by the screw press and for separating the fibers of the refoamed mass from the bubbles thereof, and means for washing the fibers separated from the refoamed mass to remove any remaining bubbles.

16. In the art of removing printing ink from paper, the step which consists in disintegrating and agitating the paper in a solution having detergent and foam producing qualities until the ink is loosened from the paper and a foamy mass is produced containing substantially no free liquid and consisting of fibers and innumerable bubbles, the particles of the ink pigment being carried by the bubbles.

17. The herein-described process of removing printing ink from paper comprising disintegrating and agitating the paper in a solution having detergent and foam producing qualities until the ink is loosened from the paper and a foamy mass is produced containing substantially no free liquid and consisting of fibers and innumerable bubbles, the particles of the ink pigment being carried by the bubbles and subjecting the foamy mass to pressure to express the bubbles with the ink pigment particles therefrom.

18. The herein described process of removing printing ink from paper which consists in disintegrating and agitating the paper in a solution having detergent and foam producing qualities and containing the foam producing constituents at least of the spent cooking liquors recovered from a digestion of fibrous vegetable material until a foamy mass is produced in which the particles of ink pigment are carried by the films of the bubbles of the foam and then expressing the bubbles with the particles thereon from the fiber.

19. In the art of treating fibrous material for the purpose of separating therefrom substances substantially insoluble in water, the steps which consist in disintegrating and agitating the material in a solution having detergent and foam producing qualities until a foamy mass is produced containing no free liquid and consisting of fiber and innumerable bubbles, particles of the substances to be separated being carried by the surfaces of the bubbles, and then expressing the bubbles with the particles thereon from the fibers.

SIDNEY D. WELLS.